# EUROPEAN PATENT SPECIFICATION

(11) **EP 1 222 316 B1**
(45) Date of publication and mention of the grant of the patent: **16.06.2004**
(21) Application number: 00961293.8
(22) Date of filing: 05.09.2000
(51) Int. Cl.: C22C 29/00, C23C 16/30, C23C 16/40, C23C 28/00, B23B 27/14

(54) **COATED CEMENTED CARBIDE INSERT**
BESCHICHTETER EINSATZ AUS ZEMENTIERTEM KARBID
PLAQUETTE EN CARBURE CEMENTE A REVETEMENT

(30) Priority: 06.09.1999 SE 9903122
(43) Date of publication of application: 17.07.2002
(73) Proprietor: Sandvik AB (publ), 811 81 Sandviken (SE)
(72) Inventor: LINDHOLM, Mikael, S-126 36 Hägersten (SE); LENANDER, Anders, S-135 53 Tyresö (SE); LINDSKOG, Per, S-125 35 Älvsjö (SE)
(74) Representative: Taquist, Lennart
(86) International application number: PCT/SE2000/001699
(87) International publication number: WO 2001/018272

(56) References cited:
- EP-A1- 0 701 982
- WO-A-98/48072
- SE-C2- 511 089
- US-A- 5 679 448
- DATABASE WPI Week 199944, Derwent Publications Ltd., London, GB; AN 1999-520900, XP002909844 & JP 11 222 665 A (NACHI FUJIKOSHI CORP) 17 August 1999

## Description

The present invention describes coated cemented carbide cutting tool inserts for the turning of stainless steels, particularly in applications with high demands of toughness behaviour. It could be for turning of stainless steels with different composition and microstructure such as austenitic, ferritic, ferriteaustenitic, superaustenitic and precipitation hardened stainless steels but also for the turning of non-stainless steels such as low carbon steels and low and medium alloyed steels.

It is well known that for cemented carbide cutting tools used in the machining of steels, the cutting edge is worn by different wear mechanisms such as chemical and abrasive wear but except for cutting data such as cutting speed, depth of cut, cutting feed rate also external cutting conditions such as use of coolant, off-centred work piece, cast skin on work piece etc. require a number of different properties of the cutting edge. The tool edge may for example fracture under a heavy intermittent cutting load resulting in so-called edge chipping. The chipping is due to lack of edge toughness. Furthermore, when turning a stainless steel, still another wear mechanism is active called adhesive wear, which is caused by the adhesive force between the stainless steel chip and the cutting edge. When the adhesive force grows large enough, edge chipping on the cutting edge will occur and, hence, the tool life will be shortened. Also when utilising a cemented carbide cutting tool for the turning of a stainless steel part when increasing the cutting speed in a stainless steel grade, the thermal energy developed in the cutting edge is considerable and the entire tool edge may plastically deform. This type of wear mechanism is known as plastic deformation wear and is in clear conflict with the edge toughness required. Hence, another requirement of the coated cemented carbide insert is that the selection of the carbide composition and the coating material results in a cutting edge exhibiting a high resistance to plastic deformation.

Commercial cemented carbide tools suitable for the machining of stainless steels are usually optimised with respect to some of the required tool properties mentioned above i.e. high resistance to mechanical, chemical, abrasive, adhesive, thermal and plastic deformation wear of a tough cemented carbide substrate coated with a wear resistant and an adherently bonded coating e.g. cemented carbide tools suitable for the turning of stainless steels SE 9602413-8 (WO-A-9720082) and milling of stainless steel SE 9901149-6 (EP-A-1038989).

Multilayer coating of the type TiₓAl₁₋ₓN or TiN-T₁₋ₓ AlxN are already known in the art as disclosed in EP-A-701982 or in WO-A-9848072.

It has now been found that excellent cutting performance in the turning of stainless steels with high toughness demands at the same time as high resistance to plastic deformation especially in heavy intermittent cutting conditions can be obtained by combination of a coated cemented carbide body comprising a WC based substrate with small additions of cubic carbides, W alloyed Co binder and with a specific grain size range of the WC grains, a specific composition range of WC+Co and a coating including an innermost, very thin layer of TiN, a second layer of TiAlN with a periodic variation of the Ti/Al ratio along the normal to the substrate/coating interface, and an outermost layer of TiN.

The cobalt binder phase is alloyed with W. The content of W in the binder phase can be expressed as the CW-ratio= M_{S} / (wt% Co * 0.0161), where M_{S} is the measured saturation magnetisation of the cemented carbide substrate in kA/m and wt% Co is the weight percentage of Co in the cemented carbide. The CW-value is a function of the W content in the Co binder phase. A high CW-value corresponds to a low W-content in the binder phase. According to the present invention improved cutting performance is achieved if the cemented carbide substrate has a CW-ratio of 0.77-0.95, preferably 0.82-0.92.

According to the present invention defined in claim 1 a turning tool insert particularly useful for difficult stainless steel turning is provided with a cemented carbide substrate with a composition of 9-12 wt% Co, preferably 10-11 wt% Co, 0.2-2.0 wt% cubic carbides, preferably 1.2-1.8 wt% cubic carbides of the metals Ta, Nb and Ti and balance WC. The cemented carbide may also contain other carbides from elements from group IVa, Va or VIa of the periodic table. The content of Ta is preferably over 0.8 wt%. The preferred average grain size of the WC at the preferred composition of 10-11 wt% Co, is 1.5-2 µm, most preferably between 1.6 and 1.8 µm. The cemented carbide may contain small amounts, <1 volume %, of η-phase (M₆C), without any detrimental effect. From the CW-value it follows that no free graphite is allowed.

The hard and wear resistant refractory coating deposited on the above described cemented carbide substrate according to the present invention comprises:
- a first (innermost) thin 0.1-0.5 µm layer of TiN
- a second layer comprising a multilayered structure of sublayers of the composition (TiₓAl₁₋ₓ)N in which x varies repeatedly between the two ranges 0.45<x<0.55 and 0.70<x<0.80. The first sublayer of (TiₓAl₁₋ₓ)N adjacent to the TiN bonding layer having an x-value in the range 0.45<x<0.55, the second sublayer of (TiₓAl₁₋ₓ)N having an x-value in the range 0.70<x<0.80 and the third sublayer having x in the range 0.45<x<0.55 and so forth repeated until 8-30 sublayers, preferably 22-24 sublayers, are formed. The thickness of this second layer comprising a multilayered structure of sublayers constitutes 75-95% of the total coating thickness. The individual sublayers of (TiₓAl₁₋ₓ)N are essentially of the same thickness but their thickness may also vary in a regular or irregular way and said sublayer thickness is found in the range of each 0.05-0.2 µm.
- a third thin at least 0.2, preferably 0.4-0.8 µm layer of (TiₓAl₁₋ₓ)N having an x-value in the range 0.45<x<0.55.
- a fourth outermost thin 0.1-0.2 µm layer of TiN.

The total thickness of the coating deposited on the cemented carbide substrate according to the present invention may vary in the range of 2-9 µm, preferably 3.5-7 µm. The layer thickness, the sublayer thickness and the coating thickness quoted above refers to measurements made close to the cutting edge, i. e. the functional part of the cutting tool.

The present invention according to claim 9 also relates to a method of making the above mentioned coated cutting tool insert comprising a WC-Co based cemented carbide body including an amount lower than 2.0 wt% of cubic carbides and with a composition of WC/Co in the range of 9-12 wt% Co, preferably 10-11 wt% Co and most preferably 10.2-10.8 wt% Co, and an amount of cubic carbides in the range of 0.2-2.0 wt%, and the balance is made up by WC. The average WC grain size is found in the range of 1.5-2.0 µm, preferably 1.6-1.8 µm.

The hard and wear resistant refractory coating is deposited onto the cemented carbide substrate by applying conventional PVD (Physical Vapor Deposition) methods and according to the present invention said coating comprises:
- a first (innermost) thin 0.1-0.5 µm bonding layer of TiN
- a second layer comprising a multilayered structure of sublayers of the composition (TiₓAl₁₋ₓ)N in which x varies repeatedly between the two ranges 0.45<x<0.55 and 0.70<x<0.80. The first sublayer of (TiₓAl₁₋ₓ)N adjacent to the TiN bonding layer having an x-value in the range 0.45<x<0.55, the second sublayer of (TiₓAl₁₋ₓ)N having an x-value in the range 0.70<x<0.80 and the third sublayer having x in the range 0.45<x<0.55 and so forth repeated until 8-30 sublayers, preferably 22-24 sublayers, are formed. The thickness of this second layer comprising a multilayered structure of sublayers constitutes 75-95% of the total coating thickness. The individual sublayers of (TiₓAl₁₋ₓ)N are essentially of the same thickness but their thickness may also vary in a regular or irregular way and said sublayer thickness is found in the range of 0.05-0.2 µm each.
- a third thin at least 0.2, preferably 0.4-0.8 µm layer of (TiₓAl₁₋ₓ)N having an x-value in the range 0.45<x<0.55.
- a fourth (outermost) thin 0.1-0.2 µm layer of TiN.

### Example 1.

A. Cemented carbide turning inserts according to the invention with the composition 10.5 wt% Co, 1.16 wt% Ta, 0.28 wt% Nb and balance made up by WC and with an average WC grain size of 1.7 µm, with a binder phase alloyed with W corresponding to a CW-ratio of 0.90, were coated with a total coating thickness of 4.5 µm by applying conventional PVD cathodic arc technique. The coating comprised a first (innermost) 0.2 µm layer of TiN followed by a 3.7 µm thick second layer comprising 23 alternating sublayers of (TiₓAl₁₋ₓ)N, where x alternatively varied between 0.5 and 0.75, and a third 0.4 µm (TiₓAl₁₋ₓ)N, where x= 0.5, and, finally, an outermost 0.2 µm layer of TiN.
B. A commercial cemented carbide turning insert with the composition 8.0 wt% Co, and balance made up by WC with an average WC grain size of 3.0 µm, with a binder phase low alloyed with W corresponding to a CW-ratio of 0.94, were coated with a 2.8 µm thick conventional multilayered CVD-coating according to the sequence TiN/TiCN/TiCN/TiN. The sublayers had approximately the same thickness.

| | | |
|---|---|---|
| Operation | Alternating axial and facial turning of an 80 mm diameter bar. | |
| Work-piece material | Austenitic stainless steel (AISI316L) | |
| Cutting speed | 160 m/min | |
| Feed rate | 0.4 mm/rev | |
| Depth of cut | 2 mm | |
| Insert-style | CNMG120408-MM | |
| Results | | Tool life (cycles): |
| Inserts A | (invention) | 5 |
| Inserts B | (prior art) | 2 |
| Comment: The main wear mechanism was plastic deformation of the cutting edge line resulting in a flank wear. Tool life criterion was flank wear >0.3 mm. | | |

### Example 2.

Inserts from A and B were tested in a turning operation.

| | | |
|---|---|---|
| Operation | Facing of a 130 mm bar with two flat sides | |
| Work-piece material | Austenitic stainless steel (SS2343) | |
| Cutting speed | 190 m/min | |
| Feed rate | 0.3 mm | |
| Depth of cut | 2 mm | |
| Insert-style | CNMG120408-MM | |
| Results | | Tool-life (cycles) |
| Inserts A | (invention) | 14 |
| Inserts B | (prior art) | 6 |
| Comment: The performance criterion was bad cutting action. The insert B shows more chipping along the cutting edge caused by more adhesion to the chips during the operation. | | |

### Example 3.

Inserts from A and B were tested in a turning operation.

| | | |
|---|---|---|
| Operation | External turning of a ring with 18 mm thickness. | |
| Work-piece material | Austenitic stainless steel (AISI316L) | |
| Cutting speed | 140 m/min | |
| Feed rate | 0.35 mm | |
| Depth of cut | 4 mm | |
| Insert-style | CNMG190616-MR | |
| Results | | Tool-life (cycles) |
| Inserts A | (invention) | 40 |
| Inserts B | (prior art) | 29 |
| Comment: The tool-life criterion was spalling on work piece caused by edge chipping due to lack of edge toughness. | | |

### Example 4.

Inserts from A and B were tested in a turning operation.

| | | |
|---|---|---|
| Operation | Longitudinal turning with Interrupted cuts. | |
| Work-piece material | Steel (SS1312) | |
| Cutting speed | 80 m/min | |
| Feed rate | 0.4 mm | |
| Depth of cut | 2 mm | |
| Insert-style | CNMG120408-MM | |
| Results | | Tool-life (minutes) |
| Inserts A | (invention) | 10 |
| Inserts B | (prior art) | 5 |
| Comment: The tool-life criterion was edge breakage. Insert A ran a full cycle. Since the difference is very big you can consider insert A to have a better toughness behaviour. | | |

### Example 5.

Inserts from A and B were tested in a turning operation.

| | | |
|---|---|---|
| Operation | Alternating facing and turning of a bar 70 mm in diameter. | |
| Work-piece material | Ferriteaustenitic steel (SAF2205) | |
| Cutting speed | 100 m/min | |
| Feed rate | 0.3 mm | |
| Depth of cut | 2 mm | |
| Insert-style | CNMG120408-MM | |
| Results | | Tool-life (cycles) |
| Inserts A | (invention) | 11 |
| Inserts B | (prior art) | 4 |
| Comment: The tool-life criterion was bad cutting action due to edge frittering, which is due to lack of edge toughness. | | |

### Example 6.

Inserts from A and B were tested in a turning operation.

| | | |
|---|---|---|
| Operation | External turning of a bar 120 mm in diameter. | |
| Work-piece material | Steel (SS2541) | |
| Cutting speed | 110 m/min | |
| Feed rate | 0.6 mm | |
| Depth of cut | 2 mm | |
| Insert-style | CNMG120408-MM | |
| Results | | Edge depression (mm) |
| Inserts A | (invention) | 0.035 |
| Inserts B | (prior art) | 0.085 |
| Comment: Tool-life criterion was predetermined time in cut (0.5 min). The depression was caused by lack of resistance to plastic deformation. | | |

## Claims

1. A coated cemented carbide cutting tool (indexable insert) for wet or dry machining, particularly for applications with high toughness demands, of stainless steels of different composition and microstructure, and of low and medium alloyed non-stainless steels, comprising a WC-Co based cemented carbide body and on said body a hard and wear resistant coating is deposited, **characterised in that** said cemented carbide body comprises a composition of 9-12 wt% Co in form of W-alloyed binder, 0.2-2.0 wt% cubic carbides from elements from group IVa, Va or VIa of the periodic table and balance WC with an average grain size of the WC is 1.5-2 µm. Further a W-alloyed binder phase with a CW-ratio in the range of 0.77-0.95 whereby CW = ratio = Mₛ/(wt% Co × 0,0161), where Mₛ is the measured saturation magnetization of the cemented carbide substrate in kA/m, and that said coating comprises
a first (innermost) thin layer of TiN
a second layer comprising a multilayered structure of each 0.05-0.2 µm thick sublayers of the composition (TiₓAl₁₋ₓ)N in which x varies repeatedly between the two ranges 0.45<x<0.55 and 0.70<x<0.80, the first sublayer of (TiₓAl₁₋ₓ)N adjacent to the TiN bonding layer having an x-value in the range 0.45<x<0.55, the second sublayer of (TiₓAl₁₋ₓ)N having an x-value in the range 0.70<x<0.80 and the third sublayer having x in the range 0.45<x<0.55 and so forth repeated until 8-30 sublayers are being built up
a third at least 0.2 µm thick layer of (TiₓAl₁₋ₓ)N, where x is found in the range 0.45<x<0.55
a fourth (outermost) thin layer of TiN making the total coating thickness vary in the range of 2-9 µm and where the thickness of the second layer constitutes 75-95% of the total coating thickness.

2. A cutting tool insert according to claim 1 **characterised in that** the Co content is within 10-11 wt%.

3. A cutting tool insert according to any of claim 1-2 **characterised in** containing 1.2-1.8 wt% cubic carbides of the metals Ta, Nb and Ti.

4. A cutting tool insert according to any of claim 1-3 **characterised in that** the content of Ta is preferably over 0.8 wt%.

5. A cutting tool insert according to any of claim 1-4 **characterised in that** the CW-ratio is 0.82-0.92.

6. A cutting tool insert according to any of claim 1-5 **characterised in that** the coating comprises of a first (innermost) thin 0.1-0.5 µm layer of TiN, a second main layer has a multilayered structure of 22-24 sublayers of the composition (TiₓAl₁₋ₓ)N in which x varies repeatedly between the two ranges 0.45<x<0.55 and 0.70<x<0.80, a third thin preferably 0.4-0.8 µm layer of (TiₓAl₁₋ₓ)N having an x-value in the range 0.45<x<0.55 and a fourth outermost thin 0.1-0.2 µm layer of TiN.

7. A cutting tool insert according to any of claim 1-6 **characterised in that** coating has a total thickness of 3.5-7 µm.

8. A cutting tool insert according to any of claim 1-7 **characterised in that** the average WC grain size is between 1.6 and 1.8 µm.

9. A method of making a cutting insert comprising a cemented carbide substrate with refractory coating according to any of the above claims **characterised in** forming a powder mixture containing WC, Co and cubic carbides
mixing said powders with pressing agent and possibly W metal such that the desired CW-ratio is obtained.
milling and spray drying the mixture to a powder material with the desired properties
pressing and sintering the powder material at a temperature of 1300-1500°C, in a controlled atmosphere of about 50 mbar followed by cooling
applying conventional post sintering treatments including edge rounding and
applying a hard, wear resistant coating by PVD-technique comprising
a first (innermost) thin layer of TiN
a second layer comprising a multilayered structure of each 0.05-0.2 µm thick sublayers of the composition (TiₓAl₁₋ₓ)N in which x varies repeatedly between the two ranges 0.45<x<0.55 and 0.70<x<0.80, the first sublayer of (TiₓAl₁₋ₓ)N adjacent to the TiN bonding layer having an x-value in the range 0.45<x<0.55, the second sublayer of (TiₓAl₁₋ₓ)N having an x-value in the range 0.70<x<0.80 and the third sublayer having x in the range 0.45<x<0.55 and so forth repeated until 8-30 sublayers are being built up
a third at least 0.2 µm thick layer of (TiₓAl₁₋ₓ)N, where x is found in the range 0.45<x<0.55
a fourth (outermost) thin layer of TiN making the total coating thickness vary in the range of 2-9 µm and where the thickness of the second layer constitutes 75-95% of the total coating thickness.

## Patentansprüche

1. Beschichtetes Hartmetallschneidwerkzeug (Wendeschneidplatte) für nasse oder trockene Bearbeitung (besonders für Anwendungen) mit der Notwendigkeit hoher Zähigkeit, von rostfreien Stählen unterschiedlicher Zusammensetzung und Mikrostruktur und von niedrig und mittelmäßig legierten nichtrostfreien Stählen mit einem Hartmetallkörper auf WC-Co-Basis und mit einer auf diesem Körper abgeschiedenen harten und verschleißfesten Beschichtung, **dadurch gekennzeichnet, daß** der Hartmetallkörper eine Zusammensetzung von 9-12 Gew.-% Co in Form von W-legiertem Bindemittel, 0,2-2,0 Gew.-% kubischen Carbiden von Eiementen aus der Gruppe IVa, Va oder VIa des Periodensystems und Rest WC, wobei eine mittlere Korngröße des WC 1,5-2 µm ist, und weiterhin mit einer W-legierten Bindephase mit einem CW-Verhältnis im Bereich von 0,77 bis 0,95, wobei CW-Verhältnis = M_{S}/(Gew.-% Co x 0,0161), worin M_{S} die gemessene Sättigungsmagnetisierung des Hartrnetallsubstrats in kA/µ bedeutet, und daß die Beschichtung
eine erste (innerste) dünne Schicht von TiN,
eine zweite Schicht, die eine mehrschichtige Struktur von jeweils 0,05-0,2 µm dicken Unterschichten der Zusammensetzung (TiₓAl₁₋ₓ)N, worin x häufig zwischen den beiden Bereichen 0,45<x<0,55 und 0,70<x<0,80 variiert, die erste Unterschicht von (TiₓAl₁₋ₓ)N in Nachbarschaft zu der TiN-Bindungsschicht einen x-Wert im Bereich von 0,45<x<0,55 hat, die zweite Unterschicht von (TiₓAl₁₋ₓ)N einen x-Wert im Bereich von 0,70<x<0,80 hat und die dritte Unterschicht x im Bereich von 0,45<x<0,55 hat usw., bis 8-30 Unterschichten aufgebaut sind,
eine dritte wenigstens 0,2 µm dicke Schicht von (TiₓAl₁₋ₓ)N, worin x sich im Bereich 0,45<x<0,55 befindet, und
eine vierte (äußerste) dünne Schicht von TiN umfaßt, was die Gesamtbeschichtungsdikke im Bereich von 2-9 µm variieren läßt und wo die Dicke der zweiten Schicht 75-95 % der gesamten Beschichtungsdicke ausmacht.

2. Schneidwerkzeugeinsatz nach Anspruch 1, **dadurch gekennzeichnet, daß** der Co-Gehalt innerhalb von 10-11 Gew.-% liegt.

3. Schneidwerkzeugeinsatz nach einem der Ansprüche 1 bis 2, **dadurch gekennzeichnet, daß** er 1,2-1,8 Gew.-% kubische Carbide der Metalle Ta, Nb und Ti enthält.

4. Schneidwerkzeugeinsatz nach einem der Ansprüche 1 bis 3, **dadurch gekennzeichnet, daß** der Gehalt an Ta vorzugsweise über 0,8 Gew.-% liegt.

5. Schneidwerkzeugeinsatz nach einem der Ansprüche 1 bis 4, **dadurch gekennzeichnet, daß** das CW-Verhältnis 0,82-0,92 beträgt.

6. Schneidwerkzeugeinsatz nach einem der Ansprüche 1 bis 5, **dadurch gekennzeichnet, daß** die Beschichtung eine erste (innerste) dünne 0,1-0,5 µm dicke Schicht von TiN umfaßt, eine zweite Hauptschicht eine mehrschichtige Struktur von 22-24 Unterschichten mit der Zusammensetzung (TiₓAl₁₋ₓ)N hat, worin x wiederholt zwischen den beiden Bereichen 0,45<x<0,55 und 0,70<x<0,80 variiert, eine dritte dünne vorzugsweise 0,4-0,8 µm dicke Schicht von (TiₓAl₁₋ ₓ)N einen x-Wert im Bereich von 0,45<x<0,55 hat und eine vierte äußerste dünne 0,1-0,2 µm dicke Schicht von TiN umfaßt.

7. Schneidwerkzeugeinsatz nach einem der Ansprüche 1-6, **dadurch gekennzeichnet, daß** die Beschichtung eine Gesamtdicke von 3,5-7 µm hat.

8. Schneidwerkzeugeinsatz nach einem der Ansprüche 1-7, **dadurch gekennzeichnet, daß** die mittlere WC-Korngröße zwischen 1,6 und 1,8 µm liegt.

9. Verfahren zur Herstellung eines Schneideinsatzes mit einem Hartmetallsubstrat mit hitzebeständiger Beschichtung nach einem der obigen Ansprüche,
**dadurch gekennzeichnet, daß** man ein Pulvergemisch bildet, das WC, Co und kubische Carbide enthält, diese Pulver mit Preßmittel und gegebenenfalls W-Metall derart vermischt, daß das erwünschte CW-Verhältnis erhalten wird,
das Gemisch zu einem Pulvermaterial mit den erwünschten Eigenschaften zermahlt und sprühtrocknet,
das Pulvermaterial bei einer Temperatur von 1300-1500 °C in einer kontrollierten Atmosphäre von etwa 50 mbar preßt und sintert und anschließend kühlt,
herkömmliche Nachsinterungsbehandlungen einschließlich Kantenabrundungen anwendet und
durch PVD-Technik eine harte, verschleißbeständige Beschichtung aufbringt, die
eine erste (innerste) dünne Schicht von TiN,
eine zweite Schicht, die eine mehrschichtige Struktur von jeweils 0,05-0,2 µm dicken Unterschichten der Zusammensetzung (TiₓAl₁₋ₓ)N, worin x häufig zwischen den beiden Bereichen 0,45<x<0,55 und 0,70<x<0,80 variiert, die erste Unterschicht von (TiₓAl₁₋ₓ)N in Nachbarschaft zu der TiN-Bindungsschicht einen x-Wert im Bereich von 0,45<x<0,55 hat, die zweite Unterschicht von (TiₓAl₁₋ₓ)N einen x-Wert im Bereich von 0,70<x<0,80 hat und die dritte Unterschicht x im Bereich von 0,45<x<0,55 hat usw., bis 8-30 Unterschichten aufgebaut sind,
eine dritte wenigstens 0,2 µm dicke Schicht von (TiₓAl₁₋ₓ)N, worin x sich im Bereich 0,45<x<0,55 befindet, und
eine vierte (äußerste) dünne Schicht von TiN umfaßt, was die Gesamtbeschichtungsdikke im Bereich von 2-9 µm variieren läßt und wo die Dicke der zweiten Schicht 75-95 % der gesamten Beschichtungsdicke ausmacht.

## Revendications

1. Outil de coupe en carbure cémenté revêtu (plaquette de coupe amovible) destinée à un usinage humide ou à sec, en particulier pour des applications requérant une forte robustesse, d'aciers inoxydables de compositions et de microstructures différentes, et d'aciers non inoxydables faiblement et moyennement alliés, comprenant un corps de carbure cémenté à base de WC-Co et sur ledit corps est déposé un revêtement dur et résistant à l'usure, **caractérisé en ce que** ledit corps de carbure cémenté comprend une composition de 9 à 12 % en poids de Co sous forme d'un liant allié à W, 0,2 à 2,0 % en poids de carbures cubiques provenant d'éléments du groupe IVa, Va ou VIa de la table périodique et le reste de WC avec une granulométrie moyenne de WC qui est de 1,5 à 2 µm ; en outre, une phase de liant alliée à W avec un rapport de CW dans la plage de 0,77 à 0,95 grâce à quoi le rapport de CW = Mₛ/( % en poids de Co x 0,0161), où Mₛ est la magnétisation à saturation mesurée du substrat de carbure cémenté en kA/m, et **en ce que** ledit revêtement comprend
une première couche mince (la plus à l'intérieur) de TiN
une seconde couche comprenant une structure à couches multiples chacune des sous-couches étant d'une épaisseur de 0,05 à 0,2 µm, de composition (TiₓAl₁₋ₓ)N dans laquelle x varie de façon répétitive entre les deux plages 0,45 < x < 0,55 et 0,70 < x < 0,80, la première sous-couche de (TiₓAl₁₋ₓ)N adjacente à la couche de liaison de TiN présentant une valeur de x dans la plage 0,45 < x < 0,55, la seconde sous-couche de (TiₓAl₁₋ₓ)N présentant une valeur de x dans la plage 0,70 < x < 0,80 et la troisième sous-couche présentant une valeur de x dans la plage 0,45 < x < 0,55 et ainsi de suite en répétant jusqu'à ce 8 à 30 sous-couches soient accumulées
une troisième couche d'au moins 0,2 µm d'épaisseur de (TiₓAl₁₋ₓ)N, où x se trouve dans la plage 0,45 < x < 0,55
une quatrième couche mince (la plus à l'extérieur) de TiN, ce qui amène l'épaisseur de revêtement totale à varier dans la plage de 2 à 9 µm et où l'épaisseur de la seconde couche constitue 75 à 95 % de l'épaisseur totale du revêtement.

2. Plaquette d'outil de coupe selon la revendication 1, **caractérisée en ce que** la teneur en Co est située dans la plage de 10 à 11 % en poids.

3. Plaquette d'outil de coupe selon l'une quelconque des revendications 1 et 2, **caractérisée en ce qu'**elle contient de 1,2 à 1,8 % en poids de carbures cubiques des métaux Ta, Nb et Ti.

4. Plaquette d'outil de coupe selon l'une quelconque des revendications 1 à 3, **caractérisée en ce que** la teneur de Ta est de préférence au-dessus de 0,8 % en poids.

5. Plaquette d'outil de coupe selon l'une quelconque des revendications 1 à 4, **caractérisée en ce que** le rapport de CW est de 0,82 à 0,92.

6. Plaquette d'outil de coupe selon l'une quelconque des revendications 1 à 5, **caractérisée en ce que** le revêtement comprend une première couche mince (la plus à l'intérieur) de 0,1 à 0,5 µm de TiN, une seconde couche principale présente une structure à couches multiples de 22 à 24 sous-couches, de composition (TiₓAl₁₋ₓ)N dans laquelle x varie de façon répétitive entre les deux plages 0,45 < x < 0,55 et 0,70 < x < 0,80, une troisième couche mince de préférence de 0,4 à 0,8 µm de (TiₓAl₁₋ₓ)N présentant une valeur de x dans la plage 0,45 < x < 0,55 et une quatrième couche mince la plus à l'extérieur de TiN de 0,1 à 0,2 µm.

7. Plaquette d'outil de coupe selon l'une quelconque des revendications 1 à 6, **caractérisée en ce que** le revêtement présente une épaisseur totale de 3,5 à 7 µm.

8. Plaquette d'outil de coupe selon l'une quelconque des revendications 1 à 7, **caractérisée en ce que** la granulométrie moyenne de WC est entre 1,6 et 1,8 µm.

9. Procédé de réalisation d'une plaquette de coupe comprenant un substrat de carbure cémenté avec un revêtement réfractaire selon l'une quelconque des revendications ci-dessus
**caractérisé par** la formation d'un mélange en poudre contenant WC, Co et des carbures cubiques
le mélange desdites poudres avec un agent de pressage et éventuellement un métal de W tel que le rapport CW désiré soit obtenu,
le broyage et le séchage par pulvérisation du mélange jusqu'à un matériau en poudre présentant lés propriétés désirées,
le pressage et le frittage du matériau en poudre à une température de 1 300 à 1 500 °C sous atmosphère contrôlée d'environ 50 mbar, suivi d'un refroidissement,
l'application de traitements post frittage classiques comprenant un émoussage des arêtes et
l'application d'un revêtement dur, résistant à l'usure par une technique de dépôt physique en phase vapeur comprenant
une première couche mince (la plus à l'intérieur) de TiN,
une seconde couche comprenant une structure à couches multiples chacune des sous-couches étant d'une épaisseur de 0,05 à 0,2 µm, de composition (TiₓAl₁₋ₓ)N dans laquelle x varie de façon répétitive entre les deux plages 0,45 < x < 0,55 et 0,70 < x < 0,80, la première sous-couche de (TiₓAl₁₋ₓ)N adjacente à la couche de liaison de TiN présentant une valeur de x dans la plage 0,45 < x < 0,55, la seconde sous-couche de (TiₓAl₁₋ₓ)N présentant une valeur de x dans la plage 0,70 < x < 0,80 et la troisième sous-couche présentant une valeur de x dans la plage 0,45 < x < 0,55 et ainsi de suite en répétant jusqu'à ce 8 à 30 sous-couches soient accumulées,
une troisième couche d'au moins 0,2 µm d'épaisseur de (TiₓAl₁₋ₓ)N, où x se trouve dans la plage 0,45 < x < 0,55,
une quatrième couche mince (la plus à l'extérieur) de TiN, ce qui amène l'épaisseur de revêtement totale à varier dans la plage de 2 à 9 µm et où l'épaisseur de la seconde couche constitue 75 à 95 % de l'épaisseur totale du revêtement.
